

## UNITED STATES PATENT OFFICE

2,110,445

## PROCESS FOR PURIFYING IMPURE LEAD

Ferdinand Leferrer, Paris, France, assignor to  
 Societe Miniere et Metallurgique de Penarroya,  
 Paris, France, a corporation of France

No Drawing. Application October 25, 1935. Serial No. 46,826. In France November 2, 1934

7 Claims. (Cl. 75—78)

It is well known that most of the molten alloys give when slowly cooled a series of solid products the composition of which varies in a continuous manner from the beginning to the end of the solidification.

Only eutectic alloys do not follow this rule.

It is thus often possible to modify the composition of an alloy and to obtain a more or less complete separation of its constituents through 10 a partial solidification with a separation of the solid and liquid phases which are in presence, in well determined conditions.

This property has been used for a long time in metallurgical processes for the refining of 15 metals.

It has already been proposed to amplify this phenomenon and to render more efficient the separation of the constituents by adding to the molten alloy, prior to the partial solidification, 20 certain elements conveniently selected.

Thus, by adding a sufficient quantity of zinc to molten argentiferous lead it has been possible to obtain, by cooling in the neighbourhood of the temperature of solidification of the lead, a floating solid crust which it is easy to separate and which carries with itself the totality of the silver 25 pre-existing in the lead.

More recently it has been tried, by using additions of alkaline or earth-alkaline metals, to 30 separate the lead from its alloys and especially from copper, tin, antimony, arsenic and bismuth with which it was possibly alloyed.

It has therefore been indicated that only additions of earth-alkaline metals (calcium, magnesium or barium) made it possible to eliminate the copper, while it was preferable to use additions of sodium for separating arsenic, antimony and bismuth.

But the experiments which have been made in 40 this way have not always given the anticipated results. It has been found that sodium had no action on bismuth which could be separated only through the earth-alkaline metals (which has precisely given rise to a commercial process for 45 debismuthizing lead).

Lastly, antimony could be separated from lead by means of sodium only in alloys having a large content of antimony.

Then it has been found, according to this invention, that additions of sodium alone to impure leads in a molten condition,—containing no or only a very small proportion of zinc, but containing copper, with as the case may be, tin and/or arsenic, and/or antimony and/or precious metals,—made it possible to separate by cooling

and in the same floating crust almost the totality of the copper and as the case may be, of the tin, of the arsenic, and also eventually part of the antimony (according to the proportion of sodium used); precious metals, if any, being not 5 eliminated.

Thus, if a liquid working lead known as lead base bullion (having been freed from inclusions of matts and slags by melting and skimming at a low temperature) is treated through metallic 10 sodium, the arsenic and the copper and the tin will be eliminated in the form of a crust which will float on the upper surface of the bath.

The antimony will remain in the lead or it will be partly eliminated according to the quantity of sodium which has been added to the working lead.

Gold and silver will remain in the lead.

For carrying the process into practice metallic sodium or sodium alloys may be used. 20

The excess of sodium remaining in the lead after treatment can be eliminated by a treatment with water, steam, or by any other known process.

As a nonlimitative example of a method for 25 carrying the invention into practice, by adding to a working lead (lead base bullion) of current composition containing 0.3% of arsenic, 0.08% of tin, 0.3% of antimony, 0.05% of copper and 0.1% of silver, metallic sodium in the proportion 30 of 5 kg. of sodium for a ton of lead, there will be obtained, after skimming at a temperature of about 330° C. (626° F.) a lead containing less than 0.01% of arsenic, less than 0.005% tin and less than 0.005% of copper. 35

The content of antimony will remain of about 0.3% and the content of silver will remain of about 0.1%.

By adding to the same molten working lead a greater proportion of sodium, for instance 15 kg. 40 of sodium for a ton of lead, the arsenic content of the lead obtained after skimming will be less than 0.005%, the tin less than 0.002%, the copper content will be less than 0.002% and the antimony content will be less than or equal to 45 0.1%. The silver will remain in the lead, with a silver content of about 0.1%.

This process allows also—by adding a quantity of sodium which is sufficient for eliminating the impurities but which is not sufficient for eliminating the antimony—of purifying any lead-antimony alloy for freeing it from the impurities which it contains (arsenic, copper for instance) and obtaining practically pure lead-antimony 50 55 alloy.

It has been thus possible, for instance, to purify a lead-antimony alloy having the following composition: arsenic 0.1%, tin 0.05%, copper 0.05% and antimony 10%, by adding to the same 5 0.4% of sodium. After the known treatment, for instance with water or steam, in order to eliminate the excess of sodium, a pure antimony-containing lead has been obtained which had the following composition: antimony 9.8%, 10 arsenic 0.003%, tin 0.001%, copper 0.002%.

This process may be combined with any other known process for purifying lead.

What I claim is:

1. In a process for purifying impure leads and 15 especially work leads containing about 0.3% arsenic, about 0.3% antimony, about 0.05% copper, and about 0.1% silver, adding metallic sodium in the proportion of 5 kg. of sodium per ton of lead, skimming the dross at a temperature of 20 about 330° C., thereby obtaining a lead containing less than 0.01% arsenic, and less than 0.005% copper, the antimony and silver remaining substantially unchanged.

2. In a process for purifying impure leads and 25 especially work leads containing about 0.3% arsenic, about 0.3% antimony, about 0.05% copper, and about 0.1% silver, adding metallic sodium in the proportion of 15 kg. of sodium per ton of lead, skimming the dross at a temperature of about 30 330° C., thereby obtaining a lead having less than 0.005% arsenic, less than 0.002% copper, less than 0.1% antimony, the silver remaining substantially unchanged.

3. A process for purifying lead base bullion 35 containing a small amount of tin, from trace to about 1% arsenic, from trace to about 0.15% copper, from trace to about 1% antimony, bismuth and noble metals which consists in adding a small amount of sodium to a molten bath of said bullion, 40 allowing the bath to cool and removing simultaneously in the crust formed on the upper part of the bath all the copper, tin and arsenic present; the antimony, bismuth and noble metals remaining in the bath.

4. A process for purifying lead base bullion 45 containing a small amount of tin, from trace to

about 1% arsenic, from trace to about 0.15% copper, from trace to about 1% antimony, bismuth and noble metals which consists in adding to a molten bath of said bullion an amount of sodium greater than that necessary for eliminating 5 arsenic, tin and copper, allowing the bath to cool and removing simultaneously in the crust formed on the upper part of the bath all the copper, tin and arsenic, with a part of the antimony in relation to the excess of sodium added, the bismuth 10 and noble metals and the rest of antimony remaining in the bath.

5. The process of purifying a hard lead containing a small amount of tin, an amount of antimony of the order of about 10% and one or 15 more of the group comprising arsenic of the order of about 0.1%, copper of the order of about 0.05%, which consists in adding to a molten bath of said lead a small amount of sodium, allowing the bath to cool and removing simultaneously in the crust 20 formed on the bath all the copper, tin and arsenic present, the antimony remaining in the bath.

6. A process for purifying lead base bullion containing the usual small amounts of arsenic, copper, tin, antimony, bismuth and noble metals, 25 which consists in adding a small amount of sodium to a molten bath of said bullion, allowing the bath to cool and removing simultaneously in the crust formed on the upper part of the bath all the copper, tin and arsenic present; the antimony, bismuth and noble metals remaining in the bath.

7. A process for purifying lead base bullion containing the usual small amounts of arsenic, copper, tin, antimony, bismuth and noble metals, 35 which consists in adding to a molten bath of said bullion an amount of sodium greater than that necessary for eliminating arsenic, tin and copper, allowing the bath to cool and removing simultaneously in the crust formed on the upper part 40 of the bath all the copper, tin and arsenic, with a part of the antimony in relation to the excess of sodium added, the bismuth and noble metals and the rest of antimony remaining in the bath.

FERDINAND LEFERRER.